

1

2,879,578

## METHOD OF RUST-PROOFING CONCRETE REINFORCING ELEMENTS

Leo Torsten Ulfstedt, Söderdalje, Sweden, assignor, by mesme assignments, to Casius Corporation Limited, Montreal, Quebec, Canada

No Drawing. Application May 14, 1953  
Serial No. 355,173

Claims priority, application Sweden March 13, 1953

4 Claims. (Cl. 25—154)

This invention relates to a method of rust-proofing iron and steel reinforcing elements intended to be cast into concrete or similar structures.

For this purpose, methods of providing reinforcing elements with a coating of a mineral composition, for example by treating the elements with a cement-containing grout, silicate-containing solutions or the like, are already known. Such coatings may be very effective, but they do not give an absolute protection against rust, since they function only by preventing, more or less, owing to their tightness, the admission of oxygen to the reinforcing elements, thus retarding rust-formation.

In order to improve the rust-preventing effect of such mineral coatings, it has been proposed to admix to the coating composition potassium chromate or other soluble chromates, in the presence of which iron cannot rust, due to the passivating effect of the chromates ions on the iron. The use of such chromates has two drawbacks, however. Firstly, from the sanitary point of view the use of chromate solutions suffers from the disadvantage that the workers handling the solutions often contract very troublesome allergic diseases. Secondly, it is uncertain whether the soluble chromate remains in the rust-protective coating for a sufficient time, as it is easily spread and distributed in the concrete owing to the wandering of moisture in the reinforced concrete structure, so that the concentration of chromate ions around the irons may soon be insufficient to produce the intended effect.

According to the present invention the drawbacks and inconveniences indicated above are eliminated by adding the chromate in the form of the extremely difficultly soluble barium chromate.

The invention is based on the facts that barium sulfate is still less soluble than barium chromate, while alkali metal chromates as well as calcium chromate are easily soluble, and further that the hydraulic and other masses, into which reinforcing elements are generally embedded, generally contain sulfates, or without any inconvenience may be mixed with a small quantity of sulfates, whereby a successive conversion of the barium chromate with formation of barium sulfate and an easily soluble chromate can take place.

Consequently, in view of the fact that the mineral grout or slurry which according to the invention is used for the treatment of the reinforcing elements has had the chromate added thereto in the form of barium chromate, it will not contain chromate ions in concentrations dangerous to health. When the elements after the application of the coating thereon and drying the coating have been cast into sulfate-containing concrete, or sulfate-containing masses of similar kind, the water present in the mass (concrete), which always contains small amounts of sulfate dissolved therein, penetrates into the rust-protective coating, whereby the barium chromate contained in the coating reacts extremely slowly with the sulfate. This results in the precipitation of barium sulfate and the formation of a soluble chromate, whereby the chromate ion-

2

concentration rises to values sufficient to secure a passivation of the reinforcing irons. If the cast mass, when set, is allowed or caused to dry completely, obviously this conversion is discontinued, but at the same time also the main cause of rust-formation is eliminated, no moisture being present. If the concrete should later absorb moisture, sulfate is again capable of diffusing onto the barium chromate in the coating on the irons, whereby the chromate ion-concentration required for passivating the irons is again restored.

The content of sulfate required in the mass into which the reinforcing elements provided with a barium chromate-containing coating according to the invention are to be cast, need not be great. It has been found in the case of common cement concrete, the binder of which is Portland cement containing sulfate corresponding to 1-3%  $\text{SO}_3$ , that the reaction of the barium chromate in the coating proceeds as intended. Even if the binder of the casting mass consists of common unslaked lime, in which the  $\text{SO}_3$ -content is seldom as high as 1%, but often as low as in the neighbourhood of 0.1-0.2%, the desired effect is obtained. Should the casting mass in any case not contain sulfate corresponding to the above-mentioned concentrations, this can be compensated by the addition of a suitable quantity of sulfate, for example calcium or sodium sulfate.

The amount of barium chromate which it is required to add to the coating composition may vary within comparatively wide limits. In view of the fact that even very low chromate ion-concentrations are sufficient to produce the desired passivating effect of the reinforcement irons, and since the relatively small difference in the solubility of the barium chromate and the barium sulfate results in a very slow formation of chromate ions, even a comparatively low content of barium chromate in the coating is sufficient to secure the maintenance of the required chromate ion-concentration in the neighbourhood of the reinforcing elements for a very long period of time. Further, as already indicated above, when the cast concrete has set and its moisture content has decreased, the possibilities of the diffusion of sulfate ions as well as chromate ions are reduced, which results simultaneously in a retarded production and a retarded removal of chromate ions.

With regard to the above-mentioned facts, even a barium-chromate content of about 1%, based on the solid components in the coating composition, is often sufficient and suitable for obtaining the desired effect. However, in certain cases it may be preferable to add the barium chromate in a considerably higher concentration, especially in the case of concrete structures which are exposed to the strong influence of moisture over long periods. Thus the barium chromate content in such cases may amount to 5, 10, 20 or even 40-50% of the other solid components in the coating composition.

Apart from the content of barium chromate, the coating composition according to the invention may be composed in any suitable manner, for example as disclosed and claimed in my and Simonsson's joint prior U.S. Patents Nos. 2,591,625 and 2,611,945. The main mineral component of the composition is preferably the hydraulic cement, such as Portland cement. The coating composition may suitably also contain a hydrophilic organic colloidal binding material which at least swells in water in an amount sufficient to render the coating flexible and tough and to produce a binding action in the coating and which retards the setting of the composition so that the coating remains reactive with water and unites with concrete in which the coated reinforcing elements are subsequently embedded, as described in the above-mentioned patents. As examples of such binding agents may

be mentioned proteineous substances, such as casein and bone glue, further carbohydrates, such as dextrin, and water-soluble cellulose derivatives, for example methyl cellulose and other water-soluble esters or ethers of cellulose. In the case of steam-cured light-weight concrete the cement may also be replaced by a mixture of a reactive siliceous material, such as finely ground sand, shale-ash, fly-ash, for example, and lime which materials in the steam-curing operation react with each other forming calcium silicates, as described in the Patent No. 2,611,945.

As is well-known, common, dense cement concrete constitutes in itself a comparatively effective rust-protection for the reinforcing irons embedded therein. However, this is not the case with light-weight concrete, and for this reason the application of the invention has its greatest importance in connection with concrete of the latter kind. By "light-weight concrete" according to the application is to be understood concrete which has been produced from light aggregate together with the usual binders, as well as concrete which has been manufactured by producing pores in the concrete mass by the addition of gas-developing or foam-producing agents, independently of whether the light-weight concrete thus produced is then left to set under the influence of moisture and air, or steam-cured by means of pressure-steam, for example at an over-pressure of 8-12 kgs. In the latter case, the application of the invention has been found to be especially favourable, in so far as it has proved that the sulfate-content in steam-cured concrete is generally present in a very easily soluble form.

When carrying out the invention in practice, the mineral coating composition containing barium chromate is first prepared by mixing the components together to a homogeneous liquid, preferably aqueous suspension. The iron or steel reinforcing elements are then coated with the resulting grout or slurry in any suitable manner, for example by dipping, brushing, spraying or other methods. The coating thus applied is thereupon dried by exposing it to the air or, if it is desired to accelerate the drying, to a current of heated air of a temperature of about 30° C., for example.

The so-coated reinforcing elements are embedded in concrete, light-weight concrete or like masses and the coating is united with the concrete during setting or steam-curing and forms, when the concrete has finally set and hardened, an effective bond between the reinforcing elements and the concrete at the same time serving as an effective rust-protective for the elements, due to the presence of barium chromate therein, as indicated above.

In the following specific non-limitative examples the application of the invention is described more in detail. The parts in the examples are parts by weight.

#### Example 1

A homogenous mixture is prepared from

|                 | Parts |
|-----------------|-------|
| Portland cement | 100   |
| Barium chromate | 2     |
| Water           | 40    |

and iron or steel reinforcing elements are dipped therein. After drying of the coating the elements are cast into common concrete, consisting of Portland cement, sand, gravel and water.

#### Example 2

Iron or steel reinforcing rods are treated with a mixture of

|                                              | Parts |
|----------------------------------------------|-------|
| Water-glass solution (common market product) | 100   |
| Barium chromate                              | 50    |

When the coating has been dried, the rods are cast into

4  
a foam-concrete prepared from slag cement, fine sand, water and a foaming agent.

#### Example 3

A mixture is prepared from

|                 | Parts |
|-----------------|-------|
| Portland cement | 100   |
| Barium chromate | 20    |
| Casein          | 6     |
| Water           | 42    |

and iron or steel reinforcing elements are dipped therein. When the coating has dried, the elements are cast into a light-weight concrete prepared from Portland cement, ground quartz-containing sand, water and aluminum powder, which light-weight concrete after setting is steam-cured in autoclave at an over-pressure of 10 kgs. per sq. cm.

#### Example 4

20 Iron or steel reinforcing elements are coated with a mixture consisting of

|                                      | Parts |
|--------------------------------------|-------|
| Finely ground quartz-containing sand | 100   |
| Slaked lime                          | 25    |
| Barium chromate                      | 10    |
| A water-soluble cellulose ether      | 3     |
| Water                                | 50    |

After the coating has been dried, the elements are cast into a light-weight concrete mixture consisting of ground, unslaked lime, fly-ash, water and aluminium powder, and if desired, 1% gypsum, in a mold. After setting the reinforced concrete bodies are steam-cured in autoclave with steam at an over-pressure of 8 kgs.

#### Example 5

Iron or steam-reinforcing elements are treated with a mixture prepared from

|                 | Parts |
|-----------------|-------|
| Cement          | 100   |
| Barium chromate | 15    |
| Alcohol         | 35    |

When the coating has been dried, the elements are cast into a light-weight concrete prepared from cement, granulated blast furnace slag and water, in a mold, whereupon the setting and hardening of the concrete bodies thus produced is accelerated by exposing the bodies to a moisture-saturated atmosphere at 80° C.

What I claim is:

- 50 In the making of reinforced concrete and similar structures, wherein rust-proofed steel and iron reinforcing elements are embedded in concrete and similar masses containing small amounts of water-soluble sulfates, the process which comprises coating the reinforcing elements with a liquid grout of a mineral composition containing at least about 1% barium chromate, based on the weight of the solid components of the coating composition and about 2-20% of a hydrophilic organic colloidal binding material which at least swells in water, drying the coating before setting takes place, and surrounding the reinforcing elements with an aqueous slurry of the concrete composition, whereby the coating on the reinforcing elements sets and unites with the concrete during setting thereof, producing effective joints between the reinforcing elements and the concrete, the said barium chromate being adapted to react with the water-soluble sulfates when moisture is present in the surrounding mass to form barium sulfate and chromate ions having a passivating effect on the iron.

- 70 In the making of reinforced concrete, wherein rust-proofed steel and iron reinforcing elements are embedded in concrete containing small amounts of water-soluble sulfates, the process which comprises coating the reinforcing elements with a liquid aqueous grout of Portland cement containing at least about 1% barium chromate, based on the weight of the solid components of the coat-

ing composition, and a small proportion of casein sufficient to render the coating tough and to produce a binding action in the coating, drying the coating before it has had time to set, and embedding the so-coated reinforcing elements in a slurry of a hydraulic cement and steam-curing the cement, whereby a reinforced concrete is produced with effective joints between the reinforcing elements and the concrete, the said barium chromate being adapted to react with the water-soluble sulfates when moisture is present in the surrounding mass to form barium sulfate and chromate ions having a passivating effect on the iron.

3. In the making of reinforced steam-cured light-weight concrete, wherein rust-proofed steel and iron reinforcing elements are embedded in concrete containing small amounts of water-soluble sulfates, the process which comprises coating the reinforcing elements with a liquid aqueous grout of Portland cement containing at least about 1% barium chromate, based on the weight of the solid components in the coating composition, and a small proportion of a hydrophilic organic colloidal binding material sufficient to render the coating tough and to produce a binding action in the coating, drying the coating before it has had time to set, and embedding the so-coated reinforcing elements in a slurry of Portland cement containing a gas-producing agent in an amount sufficient to produce a porous concrete, and subjecting the whole to a curing by pressure-steam, whereby a rein-

forced porous steam-cured light-weight concrete is produced with effective joints between the reinforcing elements and the concrete, the said barium chromate being adapted to react with the water-soluble sulfates when moisture is present in the surrounding mass to form barium sulfate and chromate ions having a passivating effect on the iron.

4. The process of claim 3 wherein the liquid aqueous grout comprises approximately the following: 100 parts of Portland cement, 20 parts barium chromate, 6 parts casein, and 42 parts water, and the embedding slurry comprises approximately the following: Portland cement, ground quartz-containing sand, aluminum powder and water, and wherein the coated reinforcing elements and slurry, after setting, are steam cured at a pressure of 10 kgs. per sq. cm.

#### References Cited in the file of this patent

#### UNITED STATES PATENTS

|    |           |                        |                |
|----|-----------|------------------------|----------------|
| 20 | 96,936    | Mariner et al. -----   | Nov. 16, 1869  |
|    | 2,105,324 | Huttemann et al. ----- | Jan. 11, 1938  |
|    | 2,374,562 | Owens -----            | Apr. 24, 1945  |
|    | 2,416,064 | Patterson et al. ----- | Feb. 18, 1947  |
| 25 | 2,430,589 | Sloan -----            | Nov. 11, 1947  |
|    | 2,591,625 | Simonsson -----        | Apr. 1, 1952   |
|    | 2,611,945 | Simonsson -----        | Sept. 30, 1952 |
|    | 2,668,122 | Pitrot -----           | Feb. 2, 1954   |